# EUROPEAN PATENT APPLICATION

(11) **EP 2 385 259 A1**
(43) Date of publication of application: **09.11.2011**
(21) Application number: 10425153.3
(22) Date of filing: 06.05.2010
(51) Int. Cl.: F15B 15/14

(54) **Fluid-operated cylinder for a vehicle adapted to handle materials**

(71) Applicant: Protec Surface Technologies S.r.L., 25081 Bedizzole (BS) (IT)
(72) Inventor: Pitacco, Fabrizio, 25081 Bedizzole (Brescia) (IT); Tosti, Michele, 25081 Bedizzole (Brescia) (IT)
(74) Representative: Lunati & Mazzoni S.r.L.

(57) **Abstract**

It is provided a fluid-operated cylinder for a vehicle (2) adapted to handle material, in which said cylinder (1) has a major extension direction (1 a) and comprises at least two sections (4) having an extension direction substantially coincident with said major extension direction (1a): an outer section (4a) adapted to surround at least part of the cylinder (1), and an inner section (4b) adapted to slide along the direction (1 a) relative to the outer section (4a); and in which at least the inner section (4b) has a coating (5) including at least one outer layer (5a) of a material of high hardness, and suitable to externally coat at least one of said sections (4).

## Description

The present invention relates to a fluid-operated cylinder for a vehicle adapted to handle materials of the type pointed out in the preamble of the first claim.

The cylinder is suitable for use in a vehicle for handling material and, more specifically, in the vehicle's devices adapted to handle the material relative to the vehicle itself. It is therefore suitable to be disposed in the region of the trailers, buckets for excavators, devices for snow-tamping in ski runs or in the salt spreading means.

In particular, the cylinder is suitable for arrangement on a truck or lorry provided with a tipping body and, more specifically, it is adapted to be disposed at the body's platform enabling movement thereof.

It is known that presently lorries having a tipping body are usually employed in the building field for transport of in-bulk material such as gravel, cement, lime.

They are characterised by the presence of a mechanism adapted to tilt said body, which mechanism is usually disposed under the body. It consists of a piston, a cylinder, commonly called tipping cylinder, and a motor adapted to move a fluid, usually oil, enabling actuation of the mechanism itself.

In particular, the tipping cylinder is a telescopic cylinder which consists of a series of steel tubes, referred to as "stages" or "sections", of a progressively decreasing diameter, each of which is nested into the tube having an immediately greater diameter. Practically the cylinder is made up of an external section remaining stationary during extension of the cylinder and adapted to receive the other sections inside it; an inner section constituting the piston and driving extension and contraction of the cylinder; and, if contemplated, at least one intermediate section, the number of said intermediate sections determining the maximum elongation of the cylinder.

Therefore, when the lorry comes close to the unloading place, the above mentioned mechanism is activated and therefore the body is lifted to such an extent that the contents thereof can come out. In particular the body is rotated through about 60° relative to a pivot disposed on the end portion of the lorry, owing to elongation of the tipping cylinder. To conclude, tilting of the lorry is made possible by the piston thrust that causes the sections to come out of their housings enabling the telescopic cylinder to reach its maximum extension.

The above described known art has some important drawbacks.

In fact, the lorry's work often takes place in highly aggressive environments that can cause deterioration of the cylinder.

Said aggressiveness is due to the fact that the work environment is characterised by a high amount of suspended powders that, when they lay down on the cylinder's sections give rise to an increase in the friction between said elements and therefore to deterioration of same. In fact, the powder particles tend to be located in the contact region between two sections giving rise to abrasion of the latter by rubbing.

Aggressiveness is further due to the fact that these suspended powders could give rise to a chemically aggressive action.

In fact, most of the suspended particles consists of basic substances such as lime for example, that are particularly aggressive towards the fluid-operated cylinder.

In addition, this chemical aggressiveness is increased by the fact that often the lorry has to work in brackish environments which, as known, are aggressive towards metals.

In conclusion, deterioration of the outer surface of the sections occurs and, as a result, worsening of the performance and lifetime of the fluid-operated cylinder can take place.

These problems have been only partly solved by a chromium-plating operation, i.e. by providing coatings usually consisting of chromium.

In fact said coatings can only ensure a limited duration of the telescopic cylinder, as they are not able to ensure an appropriate protection against the action of physico-chemical agents.

Finally, these coatings usually are obtained by means of galvanic techniques and/or consist of chemical coatings that do not provide an appropriate protection against corrosion and abrasion.

Moreover, these procedures create coatings characterised by sliding properties that are not very high.

Under this situation, the technical task underlying the present invention is to conceive a fluid-operated cylinder for a vehicle adapted to handle materials which is able to substantially obviate the mentioned drawbacks.

Within the scope of this technical task it is an important aim of the invention to provide a cylinder that is able to ensure a long duration and high reliability. Another important aim of the invention is to devise a cylinder that is provided with an outer surface of high and durable resistance to rubbing and to the action of the chemical agents of the suspended particles.

A further aim of the invention is to provide a cylinder of reduced bulkiness.

A still further aim of the invention is to provide a fluid-operated cylinder that is able to ensure a low friction and high performance over the whole lifetime thereof.

A not least aim is to conceive a fluid-operated cylinder that is particularly suitable for use in lorries as the tipping cylinder thereof.

The technical task mentioned and the aims specified are achieved by a fluid-operated cylinder as claimed in the appended Claim 1.

Preferred embodiments are highlighted in the sub-claims.

The features and advantages of the invention are hereinafter clarified by the detailed description of a preferred embodiment of the invention, with reference to the accompanying drawings, in which:
**Fig. 1** shows a vehicle provided with tipping cylinders made in accordance with the invention; and
**Fig. 2** is a sectional view of a portion of said fluid-operated cylinder.

With reference to the mentioned drawings, the fluid-operated cylinder in accordance with the invention has been generally identified by reference numeral **1**.

It is suitable for use in vehicles **2** for handling material, which vehicles are usually employed in the work field and more specifically in the building field, and for instance consist of lorries with a tipping body, trailers, excavators, devices for snow-tamping of ski runs or in salt spreading means.

In detail, it is adapted to be used in a known device **3** belonging to vehicle 2 which, owing to the presence of a motor not shown in the figure, is adapted to handle the material relative to the vehicle itself. Preferably, device 3 is adapted to handle, through the action of cylinder 1, the body **2a** of a vehicle 2 on which the material has been previously loaded. Finally, the fluid-operated cylinder 1 is of the telescopic type. namely it is adapted to vary its length during operation enabling movement of body 2a.

The cylinder 1 has a tubular shape, i.e. characterised by a major extension direction **1a**. Preferably, it has a cylindrical shape and in known manner comprises at least two sections **4** having extension directions substantially coincident with the direction 1a. Alternatively, the cylinder 1 has a prismatic shape, a polyhedral shape or the like.

In conclusion, as known in the mechanical field, the term "fluid-operated cylinder" or merely "cylinder" is understood as indicating a component of any shape, a cylindrical, prismatic or similar shape for example, used for creating a relative motion between two parts.

In detail, said two sections 4 are: an external one **4a**, adapted to at least partly enclose the fluid-operated cylinder 1, and an inner one **4b** moved by device 3 and adapted to slide along said major extension direction 1 a relative to said outer section 4a.

The outer surface **4c** of at least one of said sections 4 has a multilayer coating **5**. In detail, coating 5 is obtained at least on the outer surface of the inner section 4b which, during motion of cylinder 1, slides against the inner surface of the outer section 4a.

The multilayer coating 5 comprises at least two superimposed layers **5a**, **5b** preferably laid down sequentially by high vacuum processes.

The term "high vacuum process" is understood as identifying those coating processes carried out in a vacuum chamber, i.e. characterised by a very low inner pressure. In particular the chamber where coating 5 is obtained is a high vacuum chamber.

Among the most important high vacuum processes the PVD and PECVD techniques are known. The PVC (Physical Vapour Deposition) process is for example an atomic deposition process in which the material to be laid down is evaporated from a solid phase and transferred in the vapour phase to the pieces to be coated where it lays down forming a thin film. Unlike the preceding process, the PECVD (Plasma-enhanced chemical vapour deposition) process uses a precursor already in the vapour phase, containing the chemical species to be laid down that are made available for film formation through the action of the plasma.

Coating 5 is characterised by an overall thickness advantageously included between 1 and 30 µm.

In addition, coating 5 is adapted to ensure to a section 4, a high resistance to wear and to the action of chemical agents. In addition it is adapted to ensure a low friction between sections 4 and preferably provides self-lubricating features to the coated parts. Therefore at least the outermost layer 5a of coating 5 contains materials of high hardness such as in particular the ceramic or covalent compounds, for instance the carbon compounds like carbides, carbonitrides or oxycarbonitrides, or nano particles of various nature.

The outer layer 5a preferably contains carbon. In particular, it is a layer of DLC (Diamond like carbon). The DLC is a carbon-based material with an amorphous structure exhibiting some of the diamond features and is characterised by specific chemical bonds of the sp3 type.

The layer adjacent to the outer one 5a, i.e. the inner layer 5b, is adapted to ensure adhesion between the outer layer 5a and a section 4. In addition this layer 5b helps in improving the anticorrosive and tribologic properties of coating 5.

The inner layer 5b therefore consists of a material adapted to perform the above function such as silicon carbide, pure metal, nitrided metal, carbonitrided metal or a combination thereof.

The fluid-operated cylinder 1 in known manner can include at least one intermediate section 4d adapted to be disposed between the outer section 4a and inner section 4b, as shown in Fig. 2. The intermediate section 4d is suitable to slide relative to the outer section 4a moved by the inner section 4b owing to the particular geometry of the two sections 4b and 4d. It has the above mentioned coating 5 on the outer surface 4c, which coating is characterised by its outermost layer made of DLC.

Operation of a fluid-operated cylinder 1 described above as to its structure is the following.

When vehicle 2 comes close to the unloading area, activation of device 3 is carried out.

In detail, device 3 actuates the fluid-operated cylinder 1 which, starting to increase its length, causes rotation of body 2a thus enabling the material loaded therein to begin coming out.

In greater detail, device 3 due to the presence of the motor, pushes a fluid, usually oil under pressure, which exerts a force on the inner section 4b causing movement of said section along the direction 1a. The inner section 4b, first surrounded by the outer section 4a, therefore starts coming out from said outer section 4a and, simultaneously, drags along with it the section 4d, if any. Said motion terminates when the cylinder 1 has reached its maximum extension, i.e. when the intermediate 4d and inner 4b sections have the respective outer surfaces 4c almost fully in sight.

When unloading of the material from body 2a has been completed, the cylinder 1 driven by device 3, comes back to the starting position.

The invention comprises a new process for manufacturing a fluid-operated cylinder 1 for a vehicle adapted to handle material.

The process comprises a known starting manufacturing step in which the sections 4 are created using techniques involving extrusion, removal of chips, casting or other similar techniques.

Once sections 4 have been made, the process contemplates that at least the inner section 4b will be submitted to a series of deposition steps carried out in sequence or, alternatively, substantially simultaneously and during which coating 5 is obtained. Preferably said series of deposition steps is also applied to the intermediate section 4d and, in particular, all sections 4 are submitted to deposition.

The series of steps involves at least two deposition steps in each of which a coating layer 5 is made. In addition, at least one of the deposition steps forms on the outer surface 4c, a layer of high-hardness materials such as in particular ceramic or covalent compounds and for instance carbon compounds like carbides, carbonitrides or oxycarbonitrides, or nano particles of various nature. In particular the layer thus made is a DLC layer.

In particular, said deposition step of the DLC layer is the last one of the above mentioned series so that the last outermost layer of coating 5 is the one made of DLC.

Finally, the step preceding that for making the DLC layer creates a layer of material adapted to ensure adhesion of the DLC layer to the underlying material. In addition this layer of material improves the anticorrosive and tribologic features of coating 5.

Said series of deposition steps carried out in PVD and/or PECVD plants, can take place in one or more chambers suitably modified or expressly made. Furthermore, in the deposition steps it is possible to combine, during manufacture of a coating 5, different PVD and/or PECVD techniques in a joint or separated manner. It is also possible to vary the density, thickness and composition of coating 5 by changing the deposition duration of each individual layer during the process.

The invention enables important advantages to be achieved.

In fact, the fluid-operated cylinder thus made is characterised by a high resistance to mechanical corrosion, i.e. due to wear, and chemical corrosion, owing to the presence of the DLC layer which is inert to the action of chemical agents such as acids, bases, solvents.

Moreover, said layer 5a made of DLC allows high sliding features to be obtained due to the low coefficient of friction and the self-lubricating properties belonging to the DLC.

Therefore vehicle 2 is adapted to work in any work environment without running the risk of deteriorating cylinder 1.

A further advantage resides in the high reliability of cylinder 1 and, as a result, of vehicle 2.

Moreover coating 5 and in particular the final DLC layer allow accomplishment of a cylinder 1 of reduced bulkiness although of high strength and duration. Another advantage is represented by a reduction in costs and a less strong environmental impact due to the DLC layer.

Also important is the good repeatability of the described coating process.

The invention is susceptible of variations all falling within the scope of the inventive idea.

All of the details can be replaced by equivalent means and the materials, shapes and sizes can be of any nature and magnitude.

## Claims

1. A fluid-operated cylinder (1) for a vehicle (2) adapted to handle material, said cylinder (1) having a major extension direction (1a) and comprising at least two sections (4) having an extension direction substantially coincident with said major extension direction (1a); said sections (4) including an outer section (4a) adapted to surround at least part of said cylinder (1), and an inner section (4b) adapted to slide along said major extension direction (1a) relative to said outer section (4a), **characterised in that** at least said inner section (4b) has a coating (5) including at least one outer layer (5a) of a material of high hardness, made under high-vacuum conditions and suitable to externally coat at least one of said sections (4).

2. A cylinder (1) as claimed in claim 1, wherein said outer layer (5a) is made of DLC.

3. A cylinder (1) as claimed in claim 2, wherein said coating (5) comprises an inner layer (5b) placed between said section (4) and outer layer (5a), and adapted to ensure adhesion between said outer layer (5a) and section (4).

4. A cylinder (1) as claimed in one or more of the preceding claims, wherein each of said sections (4) is provided with said coating (5).

5. A cylinder (1) as claimed in one or more of the preceding claims, comprising at least one intermediate section (4d) adapted to be disposed between said inner section (4b) and outer section (4a), which intermediate section (4d) is movable relative to said fixed section (4a) and is provided with said coating (5).

6. A cylinder (1) as claimed in one or more of the preceding claims, wherein said coating (5) has a thickness included between 1 µm and 30 µm.

7. A cylinder (1) as claimed in one or more of the preceding claims, wherein said sections (4) are of prismatic shape.

8. A cylinder (1) as claimed in one or more of claims 1-6, wherein said sections (4) are of cylindrical shape.

9. Vehicles (2) for handling material, comprising a device (3) adapted to handle material with respect to said vehicle (2) and including a cylinder (1) as claimed in one or more of the preceding claims.

10. A process for manufacturing a fluid-operated cylinder (1) for a vehicle (2) adapted to handle material, said cylinder (1) comprising at least two sections (4) adapted to be mutually moved, said process being **characterised in that** it comprises a series of deposition steps under high-vacuum conditions forming a multilayer coating (5) covering the outer surface (4c) of at least one of said sections (4).

11. A process as claimed in claim 10, wherein one of said deposition steps forms a layer of high-hardness material.

12. A process as claimed in claim 11, wherein the last alone of said deposition steps forms said layer of high-hardness material.

13. A process as claimed in one or more of claims 10-12, wherein said series of deposition steps is carried out in a plurality of chambers.
